

March 8, 1938.

G. S. BABCOCK

2,110,496

SUBBING PHOTOGRAPHIC FILM

Filed Feb. 26, 1936

*Fig.1.*



*Fig.2.*



*Fig.3.*



*George S. Babcock,*  
INVENTOR:

*Milton M. Persina  
R. Frank Smith*  
ATTORNEYS.

BY

## UNITED STATES PATENT OFFICE

2,110,496

## SUBBING PHOTOGRAPHIC FILM

George S. Babcock, Rochester, N. Y., assignor, by  
mesne assignments, to Eastman Kodak Com-  
pany, Jersey City, N. J., a corporation of New  
Jersey

Application February 26, 1936, Serial No. 65,873

## 10 Claims.

(Cl. 95—8)

This invention relates to photographic ma-  
terials, and, more particularly, to methods for  
applying light sensitive emulsions to cellulose  
organic ester film supports.

5 It is well known that a gelatino-silver halide  
emulsion cannot be applied directly to a cellulose  
organic derivative film support. A number of  
intermediate or sublayers must be applied be-  
tween the support and the emulsion and each of  
10 these layers must adhere to the layer adjoining  
it. The degree of adhesion of the layers must be  
properly controlled in order to avoid the forma-  
tion of a product which is brittle or in which  
the layers peel from the support. If the adhesion  
15 is too great, the film is brittle and the layers crack  
when the film is bent. If the adhesion is too  
slight the layers are likely to peel or strip from  
the support when the film is treated in the de-  
veloping or fixing baths or when it is dried after  
20 such treatment.

One method of avoiding these undesirable re-  
sults in a photographic film is to coat the cellulose  
organic derivative support with a layer of an-  
other ester, such as cellulose nitrate, to which  
25 the gelatin or other subcoating layers may be  
made to adhere. This method, however, has the  
disadvantage that it introduces an inflammable  
material into the film and produces a product  
which, in many cases, does not meet the require-  
30 ments of the fire underwriters.

In the prior application of H. LeB. Gray, Serial  
No. 2,081, filed January 16, 1935, a method has  
been proposed for subbing cellulose organic ester  
35 layers which comprises applying, for example, to  
a cellulose acetate propionate film base, suc-  
cessively hydrolyzed layers of cellulose acetate pro-  
pionate. One of the more hydrolyzed layers thus  
40 applied is of a composition to which a gelatin sub-  
bing solution can be made to adhere, whereas the  
gelatin layer would not adhere to a less hydrolyzed  
ester. This method requires the application of  
at least three undercoating or sublayers to the  
45 support.

It is an object of the present invention to over-  
come the above mentioned prior art difficulties  
and to provide a method for reducing the number  
of sublayers required to affix a gelatin emulsion  
to a cellulose organic derivative film base. An-  
50 other object is to provide a subbing method which  
avoids the use of cellulose nitrate or other in-  
flammable material in a photographic film. A  
further object is to provide a subbing method  
which does not result in a brittle product or one  
55 having loosely adhering layers. Other objects

will appear from the following description of my  
invention.

I have found that a layer of a cellulose or-  
ganic ester may be applied to a cellulose organic  
ester film base to which it would not ordinarily  
5 adhere by mixing with it a synthetic resin, such  
as acetone soluble glyceryl phthalate. I have  
also found that the subbing properties of a cel-  
lulose organic ester which ordinarily adheres to  
the film base may be improved by mixing it 10  
with gelatin and a synthetic resin in proper  
amounts.

In the accompanying drawing which illustrates  
in enlarged sectional views three types of film  
made according to my invention, Fig. 1 shows a 15  
film in which a cellulose organic derivative sup-  
port is coated with a layer of hydrolyzed cellulose  
acetate and resin; Fig. 2 shows a film in which  
a cellulose acetate propionate support is coated  
with a layer of gelatin, resin, and a cellulose 20  
organic ester; and Fig. 3 shows a film similar to  
that of Fig. 1 in which both sides of the support  
are subbed and sensitized.

According to the preferred form of my inven-  
tion a film support of a cellulose organic ester, 25  
which may be cellulose acetate or cellulose ace-  
tate propionate, is coated in any suitable man-  
ner with a mixture of a hydrolyzed cellulose  
ester, such as hydrolyzed cellulose acetate, and  
a synthetic resin. The hydrolyzed ester is one 30  
which has been hydrolyzed to such an extent that  
it is not compatible with the ester of which the  
support is made and would not adhere to it. The  
resin may be any suitable synthetic resin, pos-  
sessing adhering qualities for the base such as 35  
acetone soluble glyptal or polymerized vinyl ace-  
tate. This subcoat is followed by the usual gela-  
tin layer and the sensitized emulsion layer. The  
following examples illustrate several methods of  
producing a film according to my invention. 40

## Example I

A film base of cellulose acetate propionate  
which has been slightly hydrolyzed and has a 45  
propionyl content of 16% and an acetyl con-  
tent of 29%, is lead through an immersion type  
hopper containing the following solution of cel-  
lulose acetate hydrolyzed to such an extent that  
its precipitation value is about 69%: 50

|                                    | Grams |
|------------------------------------|-------|
| Cellulose acetate                  | 6     |
| Ethyl alcohol                      | 40    |
| Acetone                            | 160   |
| Glyceryl-phthalate resin (Glyptal) | 3 55  |

This solution is coated at a linear speed of approximately three feet per minute. The film is then lead through an appropriate drying apparatus which is maintained at a temperature of approximately 120-200° F., where the solvent is evaporated from the surface of the material. The resin and ester coated material is then carried through a second immersion hopper containing a gelatin solution of approximately the following composition which is coated directly on the resin and ester layer:

|               | Grams |
|---------------|-------|
| Gelatin       | 1.2   |
| Acetic acid   | 0.12  |
| 15 Acetone    | 70    |
| Water         | 5     |
| Ethyl alcohol | 22.6  |

The gelatin coated material is then dried at appropriate temperatures after which the usual gelatin silver halide emulsion is applied upon the gel surface by known technic, thus completing the film.

#### Example II

25 A film base of cellulose acetate, which has been hydrolyzed to such an extent that its precipitation value is about 90%, is lead through an immersion type hopper containing the following cellulose acetate and resin solution in which the cellulose acetate has been hydrolyzed to such an extent that its precipitation value is about 69%:

|                              | Grams |
|------------------------------|-------|
| Hydrolyzed cellulose acetate | 6     |
| 35 Ethyl alcohol             | 40    |
| Acetone                      | 158   |
| Glyceryl-phthalate resin     | 2     |

This coating is dried and followed by the gelatin solution and gelatino-silver halide emulsion as described in the preceding example.

#### Example III

45 A fully esterified cellulose acetate propionate film base which has a precipitation value of 95-96% is lead through an immersion hopper as described in the preceding examples and is coated with the following resin and hydrolyzed cellulose acetate solution in which the cellulose acetate has a precipitation value of about 69%:

|                              | Grams |
|------------------------------|-------|
| Hydrolyzed cellulose acetate | 6     |
| Ethyl alcohol                | 40    |
| Acetone                      | 156   |
| 55 Glyceryl-phthalate resin  | 1     |

This coating is dried and followed by the gelatin solution and gelatino-silver halide emulsion as described in the preceding examples.

60 According to another modification of my invention a cellulose organic ester film base, such as slightly hydrolyzed cellulose acetate propionate, is coated with a solution of cellulose acetate propionate, which is compatible with the ester of the support, mixed with gelatin and a synthetic resin, such as a glyceryl phthalate resin. In this case this brittleness modification is accomplished by the presence of the resin in the coating, since without the resin, the film showed objectionable brittleness. This coating is dried in the usual way and is followed by a sub of gelatin and cellulose ester, and the gelatino-silver halide emulsion. The following examples illustrate a method of making a film according to this modification of my invention:

#### Example IV

A film base of a cellulose acetate propionate hydrolyzed to such an extent that the propionyl content is 16% and the acetyl content 29% is coated with a solution of cellulose acetate propionate in which the propionyl content is 17.5% and the acetyl content is 27%, the apparent acetyl content being 39%. This solution is made up in acetone and methyl alcohol or any other suitable solvent and has the following solid material content:

|                              | Per cent |
|------------------------------|----------|
| Gelatin                      | 85       |
| Cellulose acetate propionate | 12       |
| Glyceryl-phthalate resin     | 3        |

This coating is dried and is followed by a solution of gelatin and cellulose acetate propionate of the same composition as that used in the first coating and applied from any suitable solvent. 20 The solid content of this coating is as follows:

|                              | Per cent |
|------------------------------|----------|
| Gelatin                      | 85       |
| Cellulose acetate propionate | 5        |

This coating is dried in an appropriate manner and is followed by the usual gelatino-silver halide emulsion, which is coated by known technic to complete the film.

#### Example V

A film base of cellulose acetate propionate having a composition similar to that described in the preceding example is coated with a solution of hydrolyzed cellulose acetate having an 35 apparent acetyl content of 39%, mixed with gelatin and a synthetic resin. The solid content of this solution is approximately as follows:

|                              | Per cent |
|------------------------------|----------|
| Gelatin                      | 93       |
| Cellulose acetate propionate | 4        |
| Glyceryl-phthalate resin     | 3        |

This coating is followed by a coating of gelatin and cellulose acetate propionate of the same 45 composition as that used in the first coating. The solid content of this solution is approximately as follows:

|                              | Per cent |
|------------------------------|----------|
| Gelatin                      | 85       |
| Cellulose acetate propionate | 15       |

This coating is dried in an appropriate manner and coated with the usual gelatino-silver halide emulsion.

70 My invention will now be described by reference to the accompanying drawing. As illustrated therein Fig. 1 shows a film made according to the preferred embodiment of my invention in which 10 is a film support of a cellulose organic derivative and is coated with a layer 11 of a synthetic resin and a hydrolyzed cellulose ester such as hydrolyzed cellulose acetate which is incompatible with the ester of which the support is made, but compatible with the resin with which it is mixed. This layer is dried as described in the preceding examples and is followed by a gelatin layer 12 and an emulsion layer 13.

In Fig. 2 which illustrates a film formed according to the second modification of my invention in which a support 14 of cellulose acetate propionate is coated with a layer 15 of gelatin, synthetic resin, and a cellulose ester which is compatible with the ester of which the support is made. This is followed by a layer 16 of gelatin 75

and a cellulose ester and on top of this is coated the usual gelatin layer 13.

The film shown in Fig. 3 is a duplitized or double-coated film having a cellulose organic derivative support 10, layers 11 composed of hydrolyzed cellulose acetate and a synthetic resin which is compatible with the cellulose acetate, gelatin layers 12, and sensitive emulsion layers 13. This type of film is especially adapted to use in X-ray photography.

My invention is applicable to the subbing of any type of cellulose organic ester film base, such as a fully esterified or hydrolyzed mixed ester, for example, cellulose acetate propionate or cellulose acetate butyrate, or a simple ester, such as hydrolyzed cellulose acetate. The esters used in the subbing layers may also be of any composition which meets the requirements of compatibility or lack of compatibility as described above.

Among the artificial resins which may be used according to my invention, a great many materials are available. These include the polyvinyl esters, such as polymerized vinyl acetate which is known, for example, under the trade name "Gelva", the preparation of which is described in the U. S. Patents No. 1,241,738; No. 1,586,803 and No. 1,710,825. A further type of resin which may be used is the polyvinyl acetal type. These resins are condensation products of partially or completely hydrolyzed polyvinyl acetate and an aldehyde such as formaldehyde, acetaldehyde, or butyraldehyde and are known as polyvinyl acetals. They are sold under various trade names such as "Formvar", and "Alvar", the preparation of which is described in Br. Patent 351,082 and in U. S. Patents Nos. 1,955,068 and 1,990,399. A still further type of resin which I may use are the alkyd resins, which are condensation products of a poly-basic acid and a polyhydroxy alcohol. An example of this type of resin is "Glyptal", which is a condensation product of glycerin and phthalic acid or phthalic anhydride. A still further type of resin is the group known as the "Santolites" which are condensation products of formaldehyde with aromatic sulfonamides.

I have referred to the precipitation value of a number of cellulose esters in the description of my invention. Precipitation value is the customary test which is used to determine the degree to which a cellulose organic ester has been hydrolyzed. It is carried out as follows for testing a cellulose acetate:

Five grams of the dry cellulose ester are accurately weighed and placed in a wide mouth 12 oz. bottle. To this are added 100 cc. of acetone (commercial grade of 99% or better), the mixture is stirred until homogeneous. (The bottle should be closed during the stirring with a rubber stopper fitted with a shaft for the stirrer.) To this dope is added slowly from a pipette and with thorough stirring, 150 cc. of a mixture consisting of 2 parts of distilled water and 1 part acetone by volume. Care should be taken to keep the solvents and mixtures at 20° C. wherever volumes are being measured.

At the end of the addition of the acetone-water mixture, a mixture is obtained containing 40% water by volume (neglecting contraction) in which is suspended the precipitated ester. This is allowed to stand for 12 hours at 20° C. At the end of this time precipitation has reached equilibrium and proceeds no further, and during the same time settling of the precipitate occurs. 75 cc. of the clearest portion (supernatant solu-

tion) are removed with a pipette. This 25 cc. is centrifuged in stoppered bottles at high speed until the liquid is perfectly clear. Exactly 5 cc. of the clear liquid are removed with a pipette and evaporated to dryness on a tarred watch glass. If W is the weight of the residue in grams the precipitation value which equals the per cent ester precipitated,

$$=100 - \left( W \times \frac{250}{5} \times \frac{1}{5} \times 100 \right) \quad 10$$

$$=100 - 1000W$$

When this test is used for a mixed ester, such as cellulose acetate propionate, the acetone-water solution is made up so that it contains 30% of water and 70% of acetone.

The above methods of subbing produced films which have satisfactory stripping and brittleness properties when subjected to the usual tests which are described for example in my prior application Serial No. 27,409, filed June 19, 1935. The degree of adhesion of the sub layers according to my present invention is controlled by the composition of the cellulose ester and by the proportion of ester to resin. It is not necessary to rely on the strength of the solvent and its action on the film base in order to obtain layers which adhere in sufficient degree to the base. A further advantage in the use of a cellulose ester layer directly over the film base is that it seals in the plasticizer which is ordinarily contained in the film base, and therefore results in a better surface to which to apply the following gelatin-containing subbing solutions.

I claim:

1. A photographic element comprising a cellulose organic ester support, and in order thereon, a layer comprising a mixture of a synthetic resin selected from the group consisting of polyvinyl resins and alkyd resins and a hydrolyzed cellulose organic ester, a gelatin layer, and an emulsion layer.

2. A photographic element comprising a cellulose organic ester support, and in order thereon, a layer comprising a mixture of a synthetic resin selected from the group consisting of polyvinyl resins and alkyd resins and a hydrolyzed cellulose organic ester which is incompatible with the support, a gelatin layer, and an emulsion layer.

3. A photographic element comprising a cellulose organic ester support, and in order thereon, a layer comprising a mixture of a synthetic resin selected from the group consisting of polyvinyl resins and alkyd resins and a hydrolyzed cellulose organic ester, a gelatin layer, and a light-sensitive emulsion layer.

4. A photographic element comprising a cellulose organic ester support, and in order thereon, a layer comprising a mixture of a synthetic resin selected from the group consisting of polyvinyl resins and alkyd resins and a hydrolyzed cellulose organic ester which is incompatible with the support, a gelatin layer, and a light-sensitive emulsion layer.

5. A photographic element comprising a cellulose organic ester support, and in order thereon, a layer comprising a mixture of a synthetic resin selected from the group consisting of polyvinyl resins and alkyd resins and a hydrolyzed cellulose organic ester, a gelatin layer, and a gelatino-silver halide emulsion layer.

6. A photographic element comprising a cellulose organic ester support, and in order there-

on, a layer comprising a mixture of a synthetic resin selected from the group consisting of polyvinyl resins and alkyd resins and a hydrolyzed cellulose organic ester which is incompatible with the support, a gelatin layer, and a gelatino-silver halide emulsion layer.

7. A photographic element comprising a fully esterified cellulose organic ester support, and in order thereon, a layer comprising a mixture of a synthetic resin selected from the group consisting of polyvinyl resins and alkyd resins and a hydrolyzed cellulose organic ester which is incompatible with the support, a gelatin layer, and a gelatino-silver halide emulsion layer.

15 8. A photographic element comprising a cellulose organic mixed ester support, and in order thereon, a layer comprising a mixture of a synthetic resin selected from the group consisting of polyvinyl resins and alkyd resins and a hydrolyzed cellulose organic ester which is incom-

patible with the support, a gelatin layer, and a gelatino-silver halide emulsion layer.

9. A photographic element comprising a cellulose acetate propionate support, and in order thereon, a layer comprising a mixture of a synthetic resin selected from the group consisting of polyvinyl resins and alkyd resins and a hydrolyzed cellulose organic ester which is incompatible with the support, a gelatin layer, and a gelatino-silver halide emulsion layer.

10 10. A photographic element comprising a cellulose organic mixed ester support, and in order thereon, a layer comprising a mixture of a synthetic resin selected from the group consisting of polyvinyl resins and alkyd resins and a hydrolyzed cellulose acetate propionate which is incompatible with the support, a gelatin layer, and a gelatino-silver halide emulsion layer.

GEORGE S. BABCOCK. 20